

(No Model.)

D. C. RIPLEY.

ART OF DECORATING GLASSWARE.

No. 394,612.

Patented Dec. 18, 1888.

FIG. 2.



FIG. 7



WITNESSES.

Thomas W. Cawdell  
H. L. Gill.

INVENTOR.

Daniel C. Ripley

# UNITED STATES PATENT OFFICE.

DANIEL C. RIPLEY, OF PITTSBURG, PENNSYLVANIA.

## ART OF DECORATING GLASSWARE.

SPECIFICATION forming part of Letters Patent No. 394,612, dated December 18, 1888.

Application filed February 20, 1888. Serial No. 264,641. (No model.)

*To all whom it may concern:*

Be it known that I, DANIEL C. RIPLEY, of Pittsburgh, in the county of Allegheny and State of Pennsylvania, have invented a new 5 and useful Improvement in the Art of Decorating Glassware; and I do hereby declare the following to be a full, clear, and exact description thereof, reference being had to the accompanying drawings, forming part of 10 this specification, in which—

Figure 1 is a side view of a glass tumbler, on which a pattern is partially formed, this figure being designed to illustrate one stage 15 of my improved process of ornamentation. Fig. 2 is a similar view showing the completed pattern.

In forming frosted figures—such as vines, leaves, &c.—on glassware, it has been the general custom to employ a revolving wheel, 20 against which the glass is held, and which makes the necessary frosted marks or lines on it. When the pattern is formed of lines of different thicknesses, the operation is necessarily very slow, because beside the care 25 and skill required to form the whole pattern properly a considerable time is occupied in changing the wheels, several sizes of which must usually be employed before the pattern is completed, a broad-rim wheel being 30 needed to make the extended surfaces, wheels with narrower rims being necessary for the finer lines, and very small wheels being needed for the small dots of the pattern.

My invention is designed to simplify the 35 process of decoration, to save time and skilled labor, and to provide means whereby better effects can be produced than with the old style of wheel decoration.

To this end my invention consists in forming 40 a pattern on the glass in rough by means of a sand or emery blast, and then finishing it by the application of the necessary shade-lines and other fine lines by an engraving-wheel. This is a rotatory wheel, on the edge 45 of which is applied a mixture of emery and oil, which in the revolution of the wheel cuts the glass article which is held in contact therewith, producing the desired fine lines of the pattern. The engraving-wheel, being 50 fine and not subject to be blunted by wear, gives very delicate and beautiful effects, and enables the irregular or curved lines of leaf-patterns to be produced with great facility.

The glass article is held beneath the revolving engraving-wheel in contact with the lower 55 edge thereof, and the wheel being quite thin the pattern can easily be seen and followed by the workman, who is thus enabled to form it with great accuracy.

In carrying my invention into practice I 60 cut out a stencil which represents in rough the broad surfaces, spots, and thick lines of the pattern, place this on the glass, and then by means of a sand or emery blast I reproduce this pattern on the glass in the usual 65 mode, as shown in Fig. 1. This forms the main part or body of the pattern very well, the effect being better than with a wheel, because it is perfectly regular and unmarked by the streaks or striations which so often 70 appear when the wheel is used.

In order to complete the pattern, I take the glass article which is thus marked, and by holding it against a revolving engraving-wheel I form on the plain frosted surfaces 75 produced by the sand-blast the proper shade-lines and rib-lines, and in the same way I form the stems and other connecting lines of the pattern. This produces the completed 80 pattern shown in Fig. 2, which is ornate and finished, giving much better and different results than where the whole pattern is produced by means of a wheel.

The advantages of my improvement will be appreciated by those skilled in the art. 85 It results in a great saving of time, and enables the glassware to be decorated much more rapidly and with a great saving of cost.

I do not claim, broadly, the production of a pattern by means of a sand-blast, nor the 90 production of a pattern by means of a wheel; but

What I do claim is—

An improvement in the art of decorating glassware, which consists in blocking out the 95 groundwork of a pattern by a sand-blast, and finishing the said pattern by an engraving-wheel, substantially as and for the purposes described.

In testimony whereof I have hereunto set 100 my hand this 15th day of February, A. D. 1888.

DANIEL C. RIPLEY.

Witnesses:

THOMAS W. BAKEWELL,  
W. B. CORWIN.